

1,202,490.

C. DAVIS & F. KNIFFEN.  
GOLF BALL.  
APPLICATION FILED NOV. 29, 1915.

Patented Oct. 24, 1916.



Witness.  
Edwin J. Bell.

Inventors  
Cleveland Davis and  
Frederick Kniffen.  
by Wilkinson, Giusto & Mackay.

Attorneys.

# UNITED STATES PATENT OFFICE.

CLELAND DAVIS, OF THE UNITED STATES NAVY, AND FREDERICK KNIFFEN, OF WILMINGTON, DELAWARE; SAID KNIFFEN ASSIGNOR TO SAID DAVIS.

## GOLF-BALL.

1,202,490.

Specification of Letters Patent. Patented Oct. 24, 1916.

Application filed November 29, 1915. Serial No. 64,085.

To all whom it may concern:

Be it known that we, CLELAND DAVIS, Commander, U. S. Navy, and FREDERICK KNIFFEN, citizens of the United States, residing, respectively, in San Diego, California, and Wilmington, Delaware, have invented certain new and useful Improvements in Golf-Balls, (Case C;) and we do hereby declare the following to be a full, 10 clear, and exact description of the invention, such as will enable others skilled in the art to which it appertains to make and use the same.

Our invention relates to objects of an 15 elastic nature, essentially adapted for playing or sport, such as balls which are intended to be struck by clubs, bats, or similar heavy objects.

The particular embodiment of our invention is a golf ball.

The use of celluloid as a coating for golf balls has long been known. This coating is applied either in the form of a paint or varnish so as to hide the dark color of the 25 gutta-percha and make the ball itself visible on the grass of the grounds; or in the shape of cups or hemispheres of appreciable thickness which are compressed in suitably shaped presses upon the interior elastic part 30 of the ball. Balls prepared in either of these ways are liable to several objections. The painted coating of celluloid comes off and is too thin to have any effect. When the alternative method is employed, the 35 joint between the cups cannot always be made secure, as the celluloid does not always flow and fuse properly under pressure. Then, too, it is not always possible to have the ball truly centered in the cups.

40 Thirdly, air, to some extent, may be entrapped between the shoulders and the central body, and may form bubbles which collect at one side of the ball, thus throwing it out of true and interfering with its 45 ballistic properties. Fourth, celluloid,

which is a compound of a nitrate of cellulose having a low nitration index and camphor, is not very strong nor very elastic, and, moreover, is subject to change. 50 This change is accompanied by increasing brittleness on the part of the cellulose compound left behind, and sometimes a tendency to scale or crack.

We have discovered that those nitro celluloses which have a high index of nitra-

tion such as those which, under the old terminology, namely, that in which the composition of cellulose is represented by the formula  $C_6H_{10}O_5$  are called dinitro cellulose and trinitro cellulose, have a high 60 coefficient of elasticity, and are much tougher than the celluloses nitrated to a lower extent. In later terminology wherein the formula for cellulose is  $C_{24}H_{40}O_{20}$ , enannitro-cellulose  $C_{24}H_{31}O_{20}(NO_2)_9$  (Eder), 65 about typifies the preferred degree of nitration. We have found that those celluloses which have an index ranging between 11.90 and 12.30, are best in respect as to elasticity and toughness, particularly for our purpose. 70 They, however, are still somewhat too hard and brittle for use in golf balls, and they are slow in responding to a blow.

We find it desirable to modify this nitro cellulose by the addition of some emollient 75 or toughening agent. The one which we prefer to use for the purpose is castor oil. Castor oil is not liable to oxidation under any conditions, and is generally uniform in quality. We add this to the solution in 80 which nitro cellulose of the kind indicated has been dissolved. We apprehend that the acid of castor oil, namely, ricinoleic acid, is the efficient agent in this connection, and we may substitute for this oil or its acid, 85 any other corresponding fat or fatty acid, such as colza oil, corn oil, soya bean oil, rape seed oil, or their acids. Other oils of a similar character may be used. We, in fact, 90 are not restricted to vegetable oils or fats. We prefer not to use an oxidizing oil like linseed oil or tung oil, as these are apt to become resinified in the presence of oxygen. However, under the conditions of use indicated, oxidation progresses with extreme 95 slowness, when the latter oils are used, because the access of oxygen thereto is practically prevented. We may also use oils otherwise treated, such as nitrated or sulfonated oils.

We prefer to effect the formation of our golf ball cover by repeated dippings and dryings of the golf ball core or central part with its elastic rubber winding, into a suitable solution of the nitro cellulose. Other 105 means of providing a cover, such as molding into hemispheres and clamping them together, may be used, but the cover made from depositions out of solutions of the nitro cellulose and its modifying agent, the 110

castor oil, give a coating that is entirely homogeneous, particularly if in dipping, if that be the process used, the ball is immersed on the lines of different axes from time to time.

It is desirable that the solution employed should be one which will deposit, upon evaporation of the solvent, a continuous, tough, coherent coating, and preferably the 10 solvent should be one which leaves a film which has a tendency to shrink on drying. When a solvent of this kind is employed, a certain constrictive pressure is applied to the interior of the ball, and as the successive 15 coatings are applied this constriction becomes more or less cumulative, so that the interior of the ball is put under rather high compression, while the coating itself is probably in a state of tension.

20 The solvent which we find most suitable for our purpose is acetone oil, the solution employed being a somewhat viscous one. To thin the solution diluents, of course, may be employed. Other solvents might be used, 25 such as amyl acetate, which gives a very lustrous film. Methyl alcohol is not so good, as it leaves a weak film.

The label and the brambles may be produced on the coating or cover after the successive 30 dippings and dryings have been completed, by the use of a suitable press. Care must be taken in subjecting any newly covered and, consequently, somewhat tender balls to the effect of a golf ball press, that 35 the press be not too warm, as this has an apparent tendency to weaken the film.

In the drawing herewith, we have shown an enlarged sectional view of a ball of the kind we have indicated. In this, 1 is the center 40 of the core of the ball which may be any of the usual cores, such as a piece of cork; 2 is the winding of rubber strips surrounding said core; 3 is the covering of nitro cellulose; and 4 the so-called brambles on 45 the exterior of the ball formed by pressing the ball in a suitable mold, which brambles are intended to give direction to the ball in its flight.

We have found in practice that the balls 50 constructed as above, possess certain marked peculiarities. Our cover is so hard that it is not dented or scarred by the topping blows of beginners and dubs. Our cover gives the ball an elasticity which makes it respond 55 quickly and powerfully to the heavy impact of a driver, while it is dead on the green to the comparatively slighter blows of the putting iron. That is, the ball provided

with a cover made of nitrated cellulose after the manner indicated, has a latent elasticity 60 which responds only to a powerful blow but remains dormant when a lesser blow is struck. Since the higher cellulose nitrates have a high coefficient of elasticity, the ball quickly recovers from the distortion produced by a heavy blow, and this gives the ball also greater carrying power. The ball seems to hug the ground during an approaching stroke, and when struck with a high mashie shot, on striking the ground 65 at the end of the carry, the ball has little tendency to bound, but rolls rather dead 70 straight on its course.

Having thus described our invention what we claim and desire to secure by Letters 75 Patent of the United States is:

1. A golf ball having a cover comprising nitro cellulose of a high index of nitration, and a modifying agent adapted to affect its 80 toughness and elasticity.

2. A golf ball having a cover composed in part of highly nitrated nitro cellulose modified by the presence therein of a substance adapted to affect its elasticity.

3. An object comprising in its structure 85 nitro cellulose having a nitration index ranging between 11.90 and 12.30, said nitro cellulose having combined therewith an elasticity modifying agent.

4. A golf ball having a cover consisting 90 of amorphous nitro cellulose of a nitration index ranging from 11.90 to 12.30 and a fat.

5. A golf ball having a cover consisting of amorphous nitro cellulose having a high nitration index and a fat, said cover having 95 been deposited upon said ball from successive coatings of a solution of said nitro cellulose and fat in a volatile solvent, which solvent upon evaporation left said cellulose and fat deposited in a smooth, brilliant and 100 constrictive coating.

6. A playing ball having an elastic center and a cover therefor consisting of amorphous nitro cellulose having a high nitration index and a fat, said cover having been 105 deposited upon said ball from successive coatings of a solution of said nitro cellulose and castor oil in a volatile solvent, which solvent upon evaporation left said cellulose and fat deposited in a smooth, brilliant and 110 constrictive coating.

In testimony whereof, we affix our signatures.

CLELAND DAVIS.  
FREDERICK KNIFFEN.